

## UNITED STATES PATENT OFFICE

2,318,069

PROCESS OF PRODUCING SHELL FORGINGS  
AND THE LIKEStevenson Findlater, Pittsburgh, Pa., assignor to  
National Tube Company, a corporation of New  
JerseyNo Drawing. Application August 17, 1940,  
Serial No. 353,151

1 Claim. (Cl. 29—1.21)

This invention relates to producing shell forgings and the like.

In the manufacture of shell forgings and the like, a slug of proper size is heated, inserted into a die, and expanded into tight engagement with the walls thereof. The expansion is accomplished by means of a mandrel which is pushed into the die by means of a press.

In application Serial No. 312,499 filed January 5, 1940, which has matured into Patent No. 10 2,251,094, of July 29, 1941, in the name of Claude A. Witter, there is disclosed a method of making shell forgings and the like which accomplishes the foregoing with a mandrel which simultaneously forms a centering cavity. The slug is then 15 partially pierced by means of a piercing punch during which the slug is somewhat elongated by the displacement of the metal. Subsequently the thick-walled partially pierced blank is cross-rolled on a mandrel to reduce the thickness to 20 that required in the finished shell forging.

As a result of practicing this process, it has developed that while it is very rapid, the forgings cannot be so made within the tolerances specified for shell forgings. The reason for this is that both the inside and outside diameters vary and that there are helical undulations in the inside 25 surface of the forging.

It is an object of the present invention to manufacture shell forgings and the like in a rapid 30 and economical manner while eliminating the variations in the diameter and wall-thickness to obtain forgings within very close tolerances.

The foregoing and other objects will be more apparent as the following description proceeds.

According to the teachings of the present invention, a heated slug of the proper size is expanded into tight engagement with the walls of a die with the simultaneous formation of a centering cavity in the outer end thereof. This operation is performed with a mandrel of conventional design. The slug is then partially pierced to form a closed end tubular blank by the use of a piercing punch which somewhat elongates the blank by extrusion of the metal. After this the thick-walled partially pierced blank is provided with an interiorly disposed mandrel and cross-rolled 40 on a rolling mill to reduce the wall-thickness approximately, but not entirely, to that required in the finished shell forging. According to the, 50 teachings of the present invention, the cross-rolled blank with the interiorly disposed mandrel intact is then pushed through either a ring or a roller die (preferably a three-roll roller die). This final operation, by slightly reducing the out- 55

side diameter and wall-thickness of the forging, eliminates the variations in the diameter and wall-thickness which are inherent in tubular articles in which the final wall reduction is effected by cross-rolling over an interiorly disposed mandrel, and enables the production of forgings within very close tolerances.

The foregoing sequence of operations involves piercing the slug so that the bore is slightly larger than that desired in the finished product, placing a mandrel of the diameter and nose contour desired in the finished product in the pierced billet and exerting pressure on the outer end of the mandrel while the billet is being cross-rolled to reduce the wall-thickness to an amount slightly greater than that desired in the finished product, and then pushing the billet and mandrel through a die to make the final reduction in wall-thickness. It is understood, of course, that due allowance must be made in the mandrel size to compensate for shrinkage of the forging during cooling.

One of the problems of shell forging manufacture is maintaining the interior contour of the nose portion within the desired tolerances. This is overcome by pushing the mandrel into the billet and by exerting pressure on the back end of the mandrel as the billet passes through the cross-rolls which seats and keeps the point of mandrel firmly against the inner end of the billet and thus the desired nose contour is obtained. By leaving the mandrel in the billet during the final operation of pushing it through the ring or roller die this interior contour is maintained, 35 whereas, if a different mandrel is used, difficulty is had in getting a mandrel to seat or bottom in exactly the right place due to scale formation. Moreover, by leaving the mandrel in position and thereby cutting down the amount of scaling, working to closer tolerances is permitted. Also, by using the same mandrel for the two operations and using a number of mandrels in sequence, ample time is had for cooling the mandrels which would otherwise become overheated 45 if the fast cycle of operations and high output of which this method is capable were maintained.

While I have described one specific embodiment of the present invention, it will be seen that I do not wish to be limited exactly thereto, since various modifications may be made without departing from the scope of the invention, as defined by the following claim.

I claim:

The process of producing shell forgings comprising obtaining a closed end blank having a

bore of larger diameter than that desired in the finished diameter, inserting a mandrel having a diameter and contour like that desired in the finished shell forging in said bore, rolling said blank between cross-rolls to reduce the wall-thickness thereof to a slightly greater thickness than that desired in the finished product and the bore to the diameter desired in the finished product, maintaining pressure on the end of said

5 mandrel while said mandrel and blank are passing through said cross-rolls to obtain the interior nose contour desired; and subsequently pushing said reduced blank and mandrel through a die to obtain a shell forging having the desired bore diameter, interior nose contour and the desired wall-thickness.

STEVENSON FINDLATER.